

Nov. 13, 1962

H. J. RYNKIEWICZ ETAL

3,063,787

PROCESS OF WET SPINNING STEREOREGULAR POLYVINYL ALCOHOL

Filed June 17, 1960



INVENTORS

HENRY J. RYNKIEWICZ  
EUGENE W. K. SCHWARZ  
IRVING SKEIST

BY *Warburton & Cross*

ATTORNEYS

1

3,063,787

### PROCESS OF WET SPINNING STEREOREGULAR POLYVINYL ALCOHOL

Henry J. Rynkiewicz, Danbury, Conn., Eugene W. K. Schwarz, Brooklyn, N.Y., and Irving Skeist, Summit, N.J., assignors to Diamond Alkali Company, Cleveland, Ohio, a corporation of Delaware

Filed June 17, 1960, Ser. No. 36,739

9 Claims. (Cl. 18—54)

This invention relates to the production of films, fibers, threads, filaments and similar articles. More particularly, it relates to the production of such articles from polyvinyl alcohol.

It is known that polyvinyl alcohol, which is soluble in water, can be spun into fibers by wet or dry spinning methods from an aqueous solution of the resin. Such fibers, however, are characterized by their sensitivity to water, particularly to hot water. If dipped in water at normal temperature, the fiber will shrink by more than 10% of its original length, and if the temperature of the water is around 70°—90° C., the fiber will dissolve.

Polyvinyl alcohol (PVA) fibers have been made resistant to water by various methods including modification of the alcohol prior to spinning and by after-treatment of the fiber. It has been known to incorporate into the polyvinyl alcohol spinning solution a compound such as a dicarboxylic acid which is capable of forming a cross-linked structure under the influence of heat. It has also been known to acetalize the polyvinyl alcohol, then form a fiber and follow up with a heat treatment of the fiber.

Fibers, after being spun from a PVA solution, have been made resistant to water by various treatments such as stretching and heat-treating, stretching and reacting with a material such as an aldehyde, ketone or dibasic acid, exposure to formaldehyde vapors or elevated temperatures and treatment of the fiber surface with waxes, etc. Such treatments are expensive and often introduce undesirable physical characteristics and impurities in the treated fibers.

As with other types of synthetic fibers, a moderate amount of drawing or stretching orients the molecular structure and results in high tensile strength. This orientational drawing, however, is distinguished from the stretching which accompanies the aforementioned insolubilizing treatments.

2

This invention has as an object an oriented high-tensity polyvinyl alcohol fiber which, without the well-known insolubilizing treatments, is insoluble in boiling water. A further object is a method of preparing such fibers from polyvinyl alcohol resins which are substantially insoluble in boiling water. Other objects will be obvious from a careful study of the following description of this invention.

Conventional polyvinyl alcohol is obtained by saponification, hydrolysis or alcoholysis of polymerized vinyl esters, especially vinyl acetate. The molecular weight of the polyvinyl alcohol is dependent upon that of the ester, i.e., a high molecular weight polyvinyl alcohol is obtainable from an ester having a correspondingly high molecular weight. The conventional polyvinyl alcohol having a reduced viscosity of 1.0 is completely soluble in water at a temperature of about 70° C. Accordingly, an aqueous solution of polyvinyl alcohol may be employed to produce fibers, films, etc. therefrom.

The polyvinyl alcohol of this invention, hereafter referred to as "stereoregular polyvinyl alcohol" or "RPVA," is obtained by alcoholysis of polymerized vinyl halo esters, especially vinyl chloroacetates and vinyl fluoroacetates, as disclosed in U.S. patent application Ser. No. 689,768, filed October 14, 1957, and now Patent No. 2,901,341. The stereoregular polyvinyl alcohol having a reduced viscosity of 1.1 will not dissolve in water at a temperature of 100° C. RPVA may be dissolved in water at a temperature of 115°—120° C. The insolubility of stereoregular polyvinyl alcohol in water at 100° C. has been attributed to the syndiotacticity of the alcohol as contrasted to an atactic structure possessed by conventional polyvinyl alcohol.

Since pressurized equipment is necessary to maintain a water temperature in the neighborhood of 120° C., it may be desirable to employ an organic solvent to form the spinning solution. Stereoregular polyvinyl alcohol is not only insoluble in boiling water but is also insoluble in most solvents or combinations thereof. In order to determine the effect of various solvents on RPVA, a film of the material was cast from a water dispersion of the resin. The dispersion was spread on a glass plate and the water evaporated therefrom to form a film. Small sections of this film were immersed in the solvents tested and the effect of numerous solvents is shown in Table I.

TABLE I

| Reagent                          | After 5 hrs. at room temp. | After 24 hrs. at room temp. | Additional 5 hrs. at 50-55° C. | Additional 2 hrs. at 90-95° C. |
|----------------------------------|----------------------------|-----------------------------|--------------------------------|--------------------------------|
| Water                            | NNE                        | NNE                         | NNE                            | NNE                            |
| Ethylene diamine                 | Dissolved                  | Dissolved                   | Dissolved                      | Dissolved                      |
| Acetic acid, glacial             | NNE                        | NNE                         | NNE                            | NNE                            |
| Acetic anhydride                 | NNE                        | NNE                         | Considerable swelling          | Considerable swelling          |
| Ammonium thiocyanate (sat. sol.) | Considerable swelling      | Considerable swelling       | do                             | do                             |
| Formic acid (98-100%)            | do                         | do                          | do                             | do                             |
| Lithium bromide (60% sol.)       | sl. swollen                | do                          | do                             | do                             |
| Zinc chloride (60% sol.)         | NNE                        | do                          | do                             | do                             |
| Ethylene chloride                | NNE at 50° C.              | NNE at 50° C.               | NNE at 50° C.                  | NNE                            |
| Propylene carbonate              | NNE                        | NNE                         | NNE                            | NNE                            |
| 2-nitropropane                   | NNE                        | NNE                         | NNE                            | NNE                            |
| Butyrolactone                    | NNE                        | NNE                         | NNE                            | NNE                            |
| Tetrahydrofurfuryl alcohol       | NNE                        | NNE                         | NNE                            | NNE                            |
| Chloromaleic anhydride           | NNE                        | NNE                         | NNE                            | NNE                            |
| Triethylene diamine (sat. sol.)  | Apparently dissolved       | Apparently dissolved        | Apparently dissolved           | Apparently dissolved           |
| Morpholine                       | NNE                        | NNE                         | NNE                            | V. sl. swollen                 |
| N-methyl-                        | NNE                        | NNE                         | V. v. sl. swollen              | Degradation v. v. sl. swollen  |
| Piperidine                       | NNE                        | NNE                         | NNE                            | Swollen                        |
| Pyridine                         | NNE                        | NNE                         | NNE                            | NNE-darkened                   |
| Piperazine (sat. sol.)           | Appears to be dissolved    | Appears to be dissolved     | Appears to be dissolved        | Appears to be dissolved        |
| Triethanolamine                  | NNE                        | NNE                         | NNE                            | NNE                            |
| Diethanolamine                   | NNE                        | NNE                         | NNE                            | NNE                            |
| Nitroethane                      | NNE                        | NNE                         | NNE                            | NNE                            |
| Acetonitrile                     | NNE                        | NNE                         | NNE                            | NNE                            |
| N-acetylmorpholine               | NNE                        | NNE                         | NNE                            | NNE                            |
| 1,6-hexamidine—72%               | Appears to be dissolved    | Appears to be dissolved     | Appears to be dissolved        | Appears to be dissolved        |

See footnotes at end of table.

TABLE I—Continued

| Reagent                                           | After 5 hrs. at room temp. | After 24 hrs. at room temp. | Additional 5 hrs. at 50-55° C. | Additional 2 hrs. at 90-95° C. |
|---------------------------------------------------|----------------------------|-----------------------------|--------------------------------|--------------------------------|
| Resorcinol (sat. sol.)                            | Swollen                    | Considerable swelling       | Considerable swelling          | Greatly swollen.               |
| Caprolactam (sat. sol.)                           | NNE                        | V. sl. swollen              | do                             | Do.                            |
| Dimethyl sulfone (sat. sol.)                      | Sl. swollen                | Sl. swollen                 | Swollen                        | Do.                            |
| Dimethyl sulfoxide                                | Sl. swollen                | Considerable swelling       | Considerable swelling          | Do.                            |
| Tricresyl phosphate                               | NNE                        | NNE                         | NNE                            | NNE.                           |
| Chloroform                                        | NNE                        | NNE                         | NNE                            | NNE.                           |
| Sanotizer 141                                     | NNE                        | NNE                         | NNE                            | NNE.                           |
| Diacetin                                          | NNE                        | NNE                         | NNE                            | NNE.                           |
| Formamide                                         | NNE                        | Sl. swollen                 | Sl. swollen                    | Sl. swollen.                   |
| Trisooctyl phosphite                              | NNE                        | NNE                         | NNE                            | NNE.                           |
| Bis(2-ethylhexyl) hydrogen phosphate              | NNE                        | NNE                         | NNE                            | NNE.                           |
| β-Hydroxypropionitrile                            | NNE                        | NNE                         | NNE                            | Swollen.                       |
| 2-(2-aminoethylamino) ethanol                     | NNE                        | V. sl. swollen              | Appears to be dissolved        | Appears to be dissolved.       |
| 2-pyrrolidinone                                   | NNE                        | NNE                         | V. sl. swollen                 | Greatly swollen.               |
| N-methylacetamide                                 | NNE                        | NNE                         | NNE                            | Sl. swollen.                   |
| Propargyl alcohol                                 | NNE                        | V. sl. swollen              | V. sl. swollen                 | NNE.                           |
| Shell curing agent T-1                            | NNE                        | NNE                         | NNE                            | NNE.                           |
| Diglyme                                           | NNE                        | NNE                         | NNE                            | NNE.                           |
| Tetramethylene sulfone                            | NNE                        | NNE                         | NNE                            | Swollen.                       |
| β-Alanine (sat. sol.)                             | NNE                        | V. sl. swollen              | Sl. swollen                    | Do.                            |
| Glycine (sat. sol.)                               | Sl. swollen                | Swollen                     | Swollen                        | Greatly swollen.               |
| Guanylurea phosphate (sat. sol.)                  | do                         | do                          | Greatly swollen                | Appears to be dissolved.       |
| Methylamine (30% sol.)                            | Appears to be dissolved    | Appears to be dissolved     | Appears to be dissolved        | Appears to be dissolved.       |
| Methane diamine                                   | NNE                        | NNE                         | NNE                            | NNE.                           |
| β-Hydroxyethyl trimethyl ammonium bicarbonate—45% | V. sl. swollen             | V. sl. swollen              | Sl. swollen                    | Swollen.                       |
| Cyanamide (sat. sol.)                             | Considerable swelling      | Considerable swelling       | Greatly swollen                | Dissolved.                     |
| β-Propiolactone                                   | NNE                        | Greatly swollen             | Greatly swollen                | Sl. swollen.                   |
| Urea (sat. sol.)                                  | Greatly swollen            | Considerable swelling       | Considerable swelling          | Dissolved (may contain gel.).  |
| Onyx BTC-50% <sup>1</sup>                         | Considerable swelling      | Considerable swelling       | Considerable swelling          | Considerable swelling.         |
| HCl (conc.)                                       | Dissolved                  | Dissolved                   | do                             | NNE.                           |
| NH <sub>4</sub> OH (conc.)                        | Swollen                    | Swollen                     | NNE                            | (2).                           |
| SO <sub>2</sub> /dimethyl formamide, saturated    | NNE                        | NNE                         | Greatly swollen                | Greatly swollen.               |
| SO <sub>2</sub> /tetrahydrofuran, saturated       | NNE                        | NNE                         | Extremely swollen              | Extremely swollen.             |
| LiBr/dimethyl formamide, saturated                | NNE                        | Sl. swollen                 | NNE                            | (2).                           |
| LiBr/dimethyl sulfoxide, saturated                | NNE                        | NNE                         | V. v. sl. swollen              | NNE.                           |
| LiBr/tetrahydrofuran, saturated                   | NNE                        | NNE                         | Extremely swollen              | Extremely swollen.             |
| ZnCl <sub>2</sub> /dimethyl formamide, saturated  | NNE                        | NNE                         | NNE                            | Partially dissolved.           |
| ZnCl <sub>2</sub> /dimethyl sulfoxide, saturated  | V. v. sl. swollen          | Sl. swollen                 | NNE                            | (2).                           |
| ZnCl <sub>2</sub> /tetrahydrofuran, saturated     | NNE                        | NNE                         | Sl. swollen                    | Extremely swollen.             |
| Dimethyl formamide/H <sub>2</sub> O, 4:1 ratio    | V. v. sl. swollen          | Sl. swollen                 | do                             | Do.                            |
| Dimethyl sulfoxide/H <sub>2</sub> O, 4:1 ratio    | NNE                        | NNE                         | Greatly swollen                | Extremely swollen.             |
| H <sub>2</sub> O/ethylene glycol, 4:1 ratio       | Sl. swollen                | Sl. swollen                 | Extremely swollen              | Extremely swollen.             |
| Triton X-100/H <sub>2</sub> O, (conc. sol.)       | do                         | do                          | Extremely swollen              | NNE.                           |
| Diacetone alcohol                                 | Swollen                    | Greatly swollen             | Extremely swollen              | NNE.                           |
| Tetrahydropyran-2-methanol                        | NNE                        | NNE                         | NNE                            | NNE.                           |
| Ethyl carbamate                                   | NNE                        | (M.P. 48-50° C.)            | (M.P. 48-50° C.)               | NNE.                           |
| Ethylene glycol                                   | NNE                        | V. v. sl. swollen           | Sl. swollen                    | Sl. swollen.                   |
| Urea/tetrahydrofuran, saturated                   | NNE                        | NNE                         | NNE                            | Swollen.                       |
| Urea/dimethyl formamide, saturated                | NNE                        | NNE                         | Sl. swollen                    | (2).                           |
| Urea/ethylene glycol, saturated                   | NNE                        | NNE                         | do                             | Sl. swollen.                   |
| Urea/dimethyl sulfoxide, saturated                | Sl. swollen                | Extremely swollen           | Extremely swollen              | Extremely swollen.             |
| Urea/2-pyrrolidone                                | NNE                        | NNE                         | NNE                            | Extremely swollen.             |
| Cyanamide/tetrahydrofuran, saturated              | NNE                        | NNE                         | NNE                            | Extremely swollen.             |
| Cyanamide/dimethyl formamide, saturated           | NNE                        | NNE                         | V. v. sl. swollen              | Extremely swollen.             |
| Cyanamide/ethylene glycol, saturated              | NNE                        | NNE                         | NNE                            | Extremely swollen.             |
| Cyanamide/dimethyl sulfoxide, saturated           | Sl. swollen                | Extremely swollen           | Extremely swollen              | Extremely swollen.             |
| Triethylene diamine/tetrahydrofuran               | NNE                        | NNE                         | NNE                            | Extremely swollen.             |
| Triethylene diamine/dimethyl formamide            | NNE                        | NNE                         | Sl. swollen                    | Extremely swollen.             |
| Triethylene diamine/ethylene glycol               | NNE                        | NNE                         | V. sl. swollen                 | Extremely swollen.             |
| Triethylene diamine/dimethyl sulfoxide            | Sl. swollen                | Extremely swollen           | Extremely swollen              | Extremely swollen.             |
| Triethylene diamine/2-pyrrolidone                 | NNE                        | NNE                         | NNE                            | Extremely swollen.             |
| Caprolactam/tetrahydrofuran                       | NNE                        | NNE                         | NNE                            | Extremely swollen.             |
| Caprolactam/dimethyl formamide                    | NNE                        | NNE                         | Sl. swollen                    | Extremely swollen.             |
| Caprolactam/ethylene glycol                       | NNE                        | NNE                         | NNE                            | Extremely swollen.             |
| Piperazine (hydrate)/tetrahydrofuran              | NNE                        | NNE                         | Sl. swollen                    | Extremely swollen.             |
| Piperazine (hydrate)/dimethyl formamide           | NNE                        | NNE                         | NNE                            | Extremely swollen.             |
| Piperazine (hydrate)/ethylene glycol              | NNE                        | NNE                         | NNE                            | Extremely swollen.             |
| Piperazine (hydrate)/dimethyl sulfoxide           | Sl. swollen                | Extremely swollen           | Extremely swollen              | Extremely swollen.             |
| Guanylurea phosphate/tetrahydrofuran              | NNE                        | NNE                         | NNE                            | Extremely swollen.             |
| Guanylurea phosphate/dimethyl formamide           | NNE                        | NNE                         | Sl. swollen                    | Extremely swollen.             |
| Guanylurea phosphate/ethylene glycol              | NNE                        | NNE                         | do                             | Extremely swollen.             |
| Guanylurea phosphate/dimethyl sulfoxide           | Sl. swollen                | Extremely swollen           | Extremely swollen              | Extremely swollen.             |
| Dichloroacetic acid/glycerine                     | NNE                        | NNE                         | NNE                            | Extremely swollen.             |
| Dichloroacetic acid/tetrahydrofuran               | NNE                        | NNE                         | NNE                            | Extremely swollen.             |
| Dichloroacetic acid/dimethyl formamide            | NNE                        | NNE                         | V. sl. swollen                 | Extremely swollen.             |
| Dichloroacetic acid/dimethyl sulfoxide            | Extremely swollen          | Extremely swollen           | Extremely swollen              | Extremely swollen.             |
| Formic acid/ethylene glycol                       | NNE                        | NNE                         | NNE                            | Extremely swollen.             |
| Triethylamine                                     | NNE                        | NNE                         | NNE                            | Extremely swollen.             |
| Duponol WA/H <sub>2</sub> O                       | Extremely swollen          | Extremely swollen           | Extremely swollen              | Extremely swollen.             |

<sup>1</sup> Alkyl (C<sub>8</sub>-C<sub>18</sub>) dimethyl benzyl ammonium chloride—25% sol.

Note.—NNE=No noticeable effect; v.=very; sl.=slightly; conc.=concentrated; sat.=saturated; and sol.=solution.

From Table I it will be noted that ethylene diamine, saturated solution of triethylene diamine, saturated solution of piperazine, 72% solution of 1,6-hexamidine, 30% solution of methylamine and concentrated hydrochloric acid apparently dissolve the stereoregular polyvinyl alcohol. The aqueous solutions of triethylene diamine, piperazine, hexanediamine and methylamine all are quite alkaline, having a pH in the neighborhood of about 12. Films of RPVA which were reciprocated from these solutions were found to be water-soluble and this led to the belief that such materials cause a possible degradation of the alcohol, accounting for its solubility. Con-

\* Solvent boiled off.

centrated HCl is very difficult to handle and therefore is

undesirable as a solvent. For preliminary work, ethylene diamine was selected as the solvent in the preparation of the spinning solution.

Typically, a solution of stereoregular polyvinyl alcohol in ethylene diamine is extruded by means of a gear pump through a multi-hole spinnerette into a coagulating bath of methanol or other lower aliphatic alcohol containing up to four carbon atoms. From the coagulating bath the fiber or yarn is led to a positively-driven Godet and then through air to a positively-driven wind-up bobbin. By 75 adjusting the speeds of the various drives, the fiber can

be stretched or drawn in controllable amounts either in the coagulating bath or in air between the Godet and wind-up or both. It has been found advantageous to provide a heat-setting operation following the drawing which comprises immersing the fiber or passing it through a hot mineral oil bath at a temperature of about 120° to 180° C. This heat-setting operation may be accompanied by a hot-stretch operation whereby the fiber, while hot, is stretched 4 to 8 times its original length. The combination of heat and stretch not only increases the insolubility of the fiber in hot water but also orients the fiber and increases its tensile strength.

Fibers produced from water-insoluble stereoregular polyvinyl alcohol having a reduced viscosity of 1.5, in accordance with this invention, have a tenacity of at least 7.5 grams per denier. Such fibers are important in industrial uses such as cords for tires, fire hoses, industrial cords and belting, and in reinforcing fibers for many applications.

Reference has been made to the reduced viscosity ( $N_{red}$ ) of polyvinyl alcohol. This value is an indication of the molecular weight of the polymer and is equal to the specific viscosity ( $N_{sp}$ ) divided by the concentration of polymer in the solution. The flow time of the polymer solution  $t_c$  and the flow time of the solvent  $t_0$  are usually measured by the capillary method. From these values the specific viscosity is computed according to the formula

$$N_{sp} = \frac{t_0 - t_c}{t_0}$$

The reduced viscosity has a logarithmic relationship to the molecular weight of the polymer and, in general, the range is:

| $N_{red}$ | Molecular weight  |
|-----------|-------------------|
| 0.5       | 40,000-60,000     |
| 1.0-1.5   | 100,000-200,000   |
| 3.0       | 500,000-1,000,000 |

Since conventional polyvinyl alcohol is soluble in water, water generally is used as the solvent in determining the reduced viscosity. Reduced viscosity of RPVA cannot be determined in this manner, however, since it is insoluble in water. Accordingly, the reduced viscosity of the precursor, i.e., polyvinyl chloroacetates or polyvinyl fluoroacetates, is determined and, as is common practice in the polymer field, this value is assumed to be proportional to the reduced viscosity of the polyvinyl alcohol.

Denier of fibers is defined as the weight in grams of a 9,000-meter length of thread and is determined by measuring 9 meters of thread on a standard textile skeiner. The thread is removed from the skeiner and wound into a small loop about 1 inch in diameter. The loop of thread is agitated in isopropyl alcohol to remove any oil or other material which may be present on the thread surface and then air-dried. The weight of the loop in milligrams, as determined on an analytical balance, equals the denier of the sample.

Apparatus for determining tensile strength and ultimate strength consists of a triple-beam laboratory scale. To one pan of the scale is attached a #25 chain which then loops over a sprocket and hand wheel near the level of the balance, such that turning the hand wheel adds more chain to the pan of the balance, thus gradually adding weight to that pan. The second pan of the balance has a drum-type fiber clamp attached below it. Directly below this clamp is a second clamp mounted with a rack and pinion which, through a hand wheel, can raise or lower the clamp. In operating the apparatus, the chain and sliding weights on the balance are set at 0. The lower clamp is raised so that the clamps are 5 inches apart. The thread sample is clamped in the upper clamp and then pulled through the lower clamp to a point where the balance pointer reads 0 to insure that the sample is caught between clamps. The chain hand wheel is turned at a rate so as to add about 1 gram per second to the

load. At the same time the other hand wheel is turned to lower the clamp, thus keeping the balance pointer at the center mark. When the thread sample breaks, rotation of both hand wheels is stopped. At this point the sample is checked to ascertain whether the break occurred at the nip of the clamps and, if such is the case, that reading is discarded. Using the sliding weights of the balance, the weight of the chain is balanced and the reading on the scale is the breaking point. The distance the lower clamp has moved from its original position determines the ultimate stretch. The arithmetic mean of 10 breaking strength determinations is divided by the denier of the thread to give the grams per denier. The average of 10 ultimate stretch values, calculated as a percentage of 5 inches, gives the ultimate stretch percent.

Tenacity in grams per denier is converted to pounds per square inch by the formula:

$$\frac{S}{A} = 1.24 \times 10^4 \times d \times \frac{G}{D}$$

wherein:

$S$ =strength in pounds

$A$ =cross sectional area of the fiber in square inches

$d$ =density of the fiber in grams per cubic centimeter

$$\frac{G}{D} = \text{strength or tenacity in grams per denier}$$

The density of RPVA has been determined as 1.30 gr./cc. Substituting this value in the above formula, the tenacity in pounds per square inch is equal to  $16,000 \times$  grams per denier.

In order that those skilled in the art may more completely understand the present invention and the preferred methods by which the same may be carried into effect, the following specific examples are offered.

#### Example 1

A prototype laboratory spinning apparatus such as is shown schematically in the attached drawing is employed which comprises a reservoir for the spinning solution which feeds two positive displacement metering pumps which are so interconnected and are run by variable speed motor so as to permit the accurate metering of as little as  $3 \times 10^{-3}$  cc. per minute of the spinning solution. This apparatus is designed as a precision meter to extrude a uniform filament of spinning solution through the spinnerette orifice. A candle filter, using muslin as the filtering medium, is mounted in such a way as to permit the spinnerette to be raised from and lowered into the coagulating bath without interfering with the flow of spinning solution. The main purpose of the filter is to minimize the incidence of clogging of the spinnerette orifice. The spinnerette is attached to the filter through a glass tube. The coagulating bath is contained in a stainless steel tray, 24 inches long, with an effective fiber immersion length of 18 inches. Single-stretching of the fiber is effected by wrapping the fiber once around a step on a step cone, then to a rewind spool. The diameters of the steps are calculated to permit any elongation from 0 to 1000% in 50% increments. Sequential stretching is effected by two step cones mounted parallel and rotating at the same speed. The fiber is fed around the two smallest diameter steps, then around successive larger steps and is finally wound on a rewind spool. The diameters of the steps vary from  $\frac{1}{2}$  inch to 4 inches and  $\frac{1}{8}$ -inch increments, permitting up to 700% stretch by this method.

An ethylene diamine solution containing 24% stereoregular polyvinyl alcohol having a reduced viscosity of about 0.4 is extruded through the spinnerette at a rate of 1.5 feet per minute into a coagulating bath of absolute methanol. At this extrusion rate the coagulation time is 60 seconds. The fiber is subjected to a total stretch or elongation of 450% and is then dried at 130° C. for a period of 16 hours in order to remove all of the ethylene

diamine. The fiber thus produced is insoluble in boiling water.

*Example 2*

A quantity of stereoregular polyvinyl alcohol resin having a reduced viscosity of 1.5 is dissolved in ethylene diamine to provide a solution of about 10% solids. Using the apparatus of Example 1, this solution, at room temperature, is extruded through an eight-hole spinnerette at a rate of 1.5 feet per minute into a coagulating bath of absolute methanol. The RPVA fiber is stretched a total of eight times in two stages at ambient temperature, pressure and humidity. After drawing, the fiber is given a heat-setting treatment by immersion in a mineral oil bath at 130° to 160° C. for a period of 30 seconds. The fiber thus produced is an eight-filament yarn of which each filament is slightly less than one denier. This fiber is insoluble in boiling water.

Water resistance and dry tenacity of various fibers are presented in Table II:

TABLE II

| Material                                                | Water resistance                               | Tenacity, g./d. |
|---------------------------------------------------------|------------------------------------------------|-----------------|
| Conventional PVA N <sub>red</sub> 0.9 (tire cord fiber) | Insoluble in cold water, soluble in hot water. | 5-9             |
| Conventional PVA N <sub>red</sub> 1.0                   | Dissolves at 75-80° C.                         | 2-5             |
| RPVA N <sub>red</sub> 1.25                              | Insoluble in boiling water                     | 5-7.5           |
| Nylon:                                                  |                                                |                 |
| Tire cord fiber                                         |                                                | 5-8             |
| Textile fiber                                           |                                                | 4-5             |
| Rayon:                                                  |                                                |                 |
| Tire cord fiber                                         |                                                | 3-4             |
| Textile fiber                                           |                                                | 2-3             |

*Example 3*

A 10% solution of stereoregular polyvinyl alcohol in ethylene diamine is made by placing 140 grams of anhydrous ethylene diamine in a wide-mouth glass jar. To this is added a quantity of 15.5 grams of RPVA having a reduced viscosity of 1.5. The mixture is shaken vigorously to form a thin slurry and then is heated for 3 hours in a water bath at 55°-60° C. The solution is spun through a spinnerette containing 8 orifices, each of which is 0.003 inch in diameter, into an absolute methanol bath at a speed which permits approximately 45 seconds coagulation bath exposure. The strand is wet-stretched 1.5 times and wound on a supply spool. The supply spool is placed on a hot-stretch machine where the strand is passed through a bath of mineral oil maintained at a temperature of about 135-140° C. The exposure time of the strand in the bath is about 20 seconds. The amount of stretch applied to the strand is varied by changing the gear ratio of either the feed or take-off capstan wheels so that the speed of the take-off wheel is 3 to 10 times that of the feed wheel. Table III gives the properties of the fibers thus produced.

TABLE III

| Hot stretch | Denier (8 filaments) | Ultimate stretch (percent) | Tensile strength (grams) |         | Grams per denier | Pounds per sq. in. |
|-------------|----------------------|----------------------------|--------------------------|---------|------------------|--------------------|
|             |                      |                            | Range                    | Average |                  |                    |
| 3X          | 13.6                 | 13.5                       | 23.2-42.9                | 35.7    | 2.6              | 41,000             |
| 3.5X        | 12.1                 | 12.7                       | 36.2-38.5                | 37.6    | 3.1              | 50,000             |
| 4X          | 9.8                  | 10.0                       | 33.5-39.1                | 36.8    | 3.7              | 59,000             |
| 5X          | 6.9                  | 6.5                        | 25.4-29.6                | 27.7    | 4.0              | 64,000             |
| 6X          | 7.3                  | 7.2                        | 26.1-39.8                | 34.4    | 4.7              | 75,000             |
| 7X          | 6.1                  | 5.2                        | 28.0-36.9                | 32.3    | 5.3              | 85,000             |
| 8X          | 5.6                  | 6.4                        | 34.2-41.3                | 37.8    | 6.8              | 109,000            |

*Example 4*

In order to determine the effect of hot-stretch bath temperature, a 10% solution of RPVA in ethylene diamine is spun into fibers as in Example 3, except that the amount of hot-stretch is maintained at 8 times the original length

and the bath temperature is varied. Results of this test are set forth in Table IV.

TABLE IV

| 5  | Hot stretch temperature, ° C. | Thread denier | Strength (grams) |         | Grams per denier | Pounds per sq. in. | Ultimate elongation (percent) |
|----|-------------------------------|---------------|------------------|---------|------------------|--------------------|-------------------------------|
|    |                               |               | Range            | Average |                  |                    |                               |
| 10 | 134-136                       | 18.0          | 82.6-103.2       | 91.7    | 5.1              | 82,000             | 7.8                           |
|    | 157-160                       | 18.5          | 102.8-115.4      | 108.4   | 5.9              | 94,000             | 6.6                           |

*Example 5*

In order to determine the effect of size or denier per filament on physical properties, a 10% solution of RPVA in ethylene diamine is spun into filbers as in Example 3. Variation in denier is effected by changing the speed of the solution feed pump and the resultant drawdown at the spinnerette orifices. Results are set forth in Table V.

TABLE V

| 25 | Thread denier | Filament denier | Strength (grams) |         | Grams per denier | Pounds per sq. in. | Ultimate elongation (percent) |
|----|---------------|-----------------|------------------|---------|------------------|--------------------|-------------------------------|
|    |               |                 | Range            | Average |                  |                    |                               |
|    | 5.6           | 0.7             | 34.2-41.3        | 37.8    | 6.8              | 109,000            | 6.4                           |
|    | 7.6           | 0.9             | 45.0-53.2        | 48.4    | 6.4              | 103,000            | 6.4                           |
|    | 18.0          | 2.2             | 82.6-103.2       | 91.7    | 5.1              | 82,000             | 7.8                           |

*Example 6*

In order to determine the effect of varying both the hot-stretch bath temperature and monofilament size, a 10% solution of RPVA in ethylene diamine is spun into fibers as in Example 3, except that the solution is spun through a 16 orifice spinnerette. The amount of hot-stretch is maintained at 8 times the original length.

TABLE VI

| 45 | Denier      |              | Hot stretch temperature, ° C. | Tensile strength (grams) | Grams per denier | Pounds per sq. in. |
|----|-------------|--------------|-------------------------------|--------------------------|------------------|--------------------|
|    | 16 filament | Monofilament |                               |                          |                  |                    |
|    | 19.8        | 1.2          | 135-140                       | 110                      | 5.6              | 90,000             |
|    | 28.5        | 1.7          | 171-175                       | 188                      | 6.6              | 106,000            |
|    | 9.5         | 0.6          | 171-175                       | 86                       | 9.0              | 144,000            |

It is to be understood that although the invention has been described with specific reference to particular embodiments thereof, it is not to be so limited, since changes and alterations therein may be made which are within the full intended scope of this invention as defined by the appended claims.

What is claimed is:

1. The method of producing stereoregular polyvinyl alcohol fibers which are insoluble in water at 100° C. and have a tenacity of at least 6.8 grams per denier which comprises the steps of forming a solution of stereoregular polyvinyl alcohol in ethylene diamine containing about 3% to 24% by weight polyvinyl alcohol, extruding the solution through a spinnerette into a coagulating bath of lower aliphatic alcohol containing up to 4 carbon atoms, wet-stretching the fiber to about 1 to 3 times its original length and hot-stretching the fiber about 4 to 12 times its original length at a temperature of about 120°-180° C.
2. The method of claim 1 wherein the solution contains about 10% polyvinyl alcohol.
3. The method of claim 1 wherein the polyvinyl alcohol has a reduced viscosity within the range of 0.4 to 1.5.
4. The method of claim 1 wherein the coagulating bath is absolute methanol.

5. The method of claim 1 wherein the polyvinyl alcohol has a reduced viscosity of at least 1.5.

6. The method of claim 1 wherein the fiber is wet-stretched about 1.5 times its original length and is hot-stretched about 8 times its original length at a temperature in the neighborhood of 130°-160° C.

7. The method of claim 1 wherein the fiber is hot-stretched in a bath of hot mineral oil.

8. The method of producing stereoregular polyvinyl alcohol fibers which are insoluble in water at 100° C. and have a tenacity of at least 6.8 grams per denier which comprises dissolving in ethylene diamine about 10% by weight of stereoregular polyvinyl alcohol which is insoluble in boiling water and has a reduced viscosity of at least 1.2, extruding the solution through a spinnerette into a coagulating bath of lower aliphatic alcohol containing up to 4 carbon atoms, wet-stretching the fiber to about 1 to 3 times its original length and hot-stretching

10  
15

the fiber about 4 to 12 times its original length at a temperature of about 120°-180° C.

9. The method of claim 8 wherein the stereoregular polyvinyl alcohol has a reduced viscosity of about 1.5 the fiber has a denier of 0.6 denier per filament, the hot-stretch temperature is 171°-175° C. and the tenacity of the fiber is 9.0 grams per denier.

References Cited in the file of this patent

UNITED STATES PATENTS

|           |                       |                |
|-----------|-----------------------|----------------|
| 2,447,140 | Shelton et al. -----  | Aug. 17, 1948  |
| 2,517,694 | Merion et al. -----   | Aug. 8, 1950   |
| 2,610,359 | Hatchard et al. ----- | Sept. 16, 1952 |
| 2,610,360 | Cline et al. -----    | Sept. 16, 1952 |
| 2,642,333 | Tomonari et al. ----- | June 16, 1953  |
| 2,715,763 | Marley -----          | Aug. 23, 1955  |

UNITED STATES PATENT OFFICE  
CERTIFICATE OF CORRECTION

Patent No. 3,063,787

November 13, 1962

Henry J. Rynkiewicz et al.

It is hereby certified that error appears in the above numbered patent requiring correction and that the said Letters Patent should read as corrected below.

Column 2, lines 25 and 26, strike out ", and now Patent No. 2,901,341"; columns 1 and 2, TABLE I, under the column heading "Reagent" line 5, for "thiochanate" read -- thiocyanate --; same table, same column heading, line 18, for "Piperidine" read -- Piperidine --; column 3, line 72, for "reciprocated" read -- reprecipitated --; column 5, line 39, for "alcihol" read -- alcohol --; column 10, line 4, after "1.5" insert a comma.

Signed and sealed this 24th day of September 1963.

(SEAL)

Attest:

ERNEST W. SWIDER  
Attesting Officer

DAVID L. LADD  
Commissioner of Patents